# EUROPEAN PATENT SPECIFICATION

(11) **EP 0 824 227 B1**
(45) Date of publication and mention of the grant of the patent: **14.03.2001**
(21) Application number: 97113883.9
(22) Date of filing: 12.08.1997
(51) Int. Cl.: G03G 9/12, G03G 9/135, G03G 9/125

(54) **Liquid toner composition and method of manufacturing the same**
Flüssigentwicklerzusammensetzung und Verfahren zu deren Herstellung
Composition de révélateur liquide et procédé pour sa fabrication

(30) Priority: 15.08.1996 JP 21576596
(43) Date of publication of application: 18.02.1998
(73) Proprietor: Mitsubishi Heavy Industries, Ltd., Tokyo 100-0005 (JP)
(72) Inventor: Suda, Yasuharu, Mitsubishi Heavy Ind., Ltd., Nishi-ku, Hiroshima, Hiroshima-ken (JP); Kuno, Hiroaki, Mitsubishi Heavy Ind., Ltd., Nishi-ku, Hiroshima, Hiroshima-ken (JP)
(74) Representative: Gramm, Werner, Prof. Dipl.-Ing.

(56) References cited:
- EP-A- 0 224 912
- US-A- 3 939 087
- US-A- 4 058 470
- PATENT ABSTRACTS OF JAPAN vol. 95, no. 11, 26 December 1995 & JP 07 216097 A (MITSUBISHI HEAVY IND.), 15 August 1995,
- PATENT ABSTRACTS OF JAPAN vol. 18, no. 48 (P-1682), 25 January 1994 & JP 05 273792 A (DAINIPPON PRINTING), 22 October 1993,
- PATENT ABSTRACTS OF JAPAN vol. 17, no. 485 (P-1605), 2 September 1993 & JP 05 119544 A (DAINIPPON PRINTING), 18 May 1993,
- DATABASE WPI Section Ch, Week 7826 Derwent Publications Ltd., London, GB; Class G08, AN 78-46868 XP002047224 & JP 53 057 039 A (RICOH) , 24 May 1978

## Description

The present invention relates to a liquid toner composition and a method of manufacturing the same.

The conventional liquid toner composition for electrophotography comprises, for example, an electrically insulating carrier liquid, coloring particles dispersed in the carrier liquid, a resin soluble in an electrically insulating liquid and serving to disperse and fix the coloring particles, and a charge controller for charging the coloring materials positive or negative. The coloring particles contained in the composition are excellent in dispersion capability to make the toner composition excellent in resolution. However, the conventional liquid toner composition is poor in its fixing capability. Also, the agglomerating force of the coloring particles is low in the image portion. It follows that, when a picture image is transferred from a photosensitive body to a supporting sheet, the image is likely to be collapsed so as to bring about flow of the toner particles, leading to deterioration of the transferred picture image.

As a measure for overcoming the above-noted difficulty, proposed is a liquid toner composition prepared by dispersing toner particles consisting of a pigment and a resin in an electrically insulating liquid, said resin being substantially insoluble in said electrically insulating liquid. Also proposed in, for example, Japanese Patent Publication (Kokoku) No. 5-87825, is a technical idea that the toner particles are shaped to have fiber-like projections so as to increase the agglomerating force among the toner particles.

The US-Patent 5,058,470 A discloses a liquid developer composition comprising toner particles, a liquid organic solvent, a polyvinyl acetate resin and a hydrophobic colloidal silica combined with said resin.

The US-Patent 3,939,087 discloses a liquid toner comprising a pigment and a hydrocarbon carrier having a composition containing aromatic liquid constituents and silane.

EP-A-224912 discloses a process for preparation of liquid toner wherein the liquid toner comprises toner particles, thermoplastic resins and additional components like particle size oxides such as silica. The method for manufacturing a liquid toner providing the steps of dispersing a thermoplastic resin, a non-polar liquid and a colorant particles at an elevated temperature, cooling the dispersion and separating the dispersion of toner particles from the particulate media. The resins are insoluble in the dispersant liquid at temperatures below 40°C and are able to solvate at temperatures above 50°C. The dispersant liquids are having a flash point of more than 69°C.

JP-A-5119544 relates to a toner comprising pigment particles and resin particles dispersed in an electric insulating liquid. A resin is dissolved in a solvent at a temperature higher than the dissolving temperature of the resin.

JP-A-5273792 discloses a toner consisting of an resin comprising a coloring agent dissolved in a solvent.

JP-A-7216097 describes a method for producing colored polymer fine particles, wherein a polymer resin is dispersed in a nonaqueous solvent.

However, if the agglomerating force among the toner particles dispersed in a liquid is unduly high, the toner particles tend to be excessively agglomerated to form large coarse particles which are likely to be precipitated. Further, in the step of developing the electrostatic latent image formed on the surface of a photosensitive body, the presence of the agglomerated toner particles brings about reduction of resolution.

An object of the present invention is toprovide a liquid toner composition containing toner particles which do not exhibit a high agglomerating force and are excellent in dispersion capability during storage and development of the composition, and which exhibit an increased agglomerating force in the transferring step so as to suppress collapsing and flow of the picture image, leading to an improved picture image. The preseint invention is also intended to provide a method of manufacturing the particular liquid toner composition.

According to a first aspect of the present invention, there is provided a liquid toner composition, wherein particles containing a colorant and a resin as main components are dispersed in a carrier liquid, titanium oxide or titanium hydroxide is attached to or contained in a surface region of said toner particles, and the surface of said titanium oxide or titanium hydroxide is treated with an organic substance or a hydroxide.

According to a second aspect of the present invention, there is provided a method of manufacturing a liquid toner composition, comprising the step of heating, dissolving, mixing and dispersing a thermoplastic resin in a solvent that permits dissolving said thermoplastic resin when heated and is substantially incapable of dissolving the thermoplastic resin at room temperature, said solvent having a solubility parameter (SP) value adjusted for controlling the diameter of the toner particle based on a difference in SP value between the thermoplastic resin itself and the solvent, followed by cooling to permit the toner particles to be precipitated, wherin inorganic fine particles are added by at latest the stage immediately before initiation of the toner particle precipitation.

The invention can be more fully understood from the folowing detailed description when taken in conjunction with the accompanying drawings, in which:

Figure shows how to evaluate the ER property of the liquid toner composition of the present invention.

A pigment used in general for preparing an ink composition, a toner compositin, etc. can be used in the present invention as the colorant contained in the liquid toner composition. For example, a black pigment used in the present invention includes various carbon blacks inclusing all the carbon blacks prepared by, for example, a surface method, a contact method and an acetylene method and available on the market for use in the manufacture of rubber and a coloring metarial and for use as an electrically conductive material. To be more specific, classification of carbon black is given on pages 290 to 291 of "Carbon Black Binran (Manual)" published in April, 1995. The carbon black used in the present invention includes any classification of HCF, MCF, RCF, LCF, LFF, which are prepared by a furnace method, and HCC, MCC, RCC, LCC, which are prepared by a channel method. Further, various acetylene blacks given on page 294 of "Carbon Black Binran" noted above can also be used in the present invention.

The non-black pigment used in the present invention as the colorant includes, for example, phthalocyanine blue, phthalocyanine green, sky blue, rhodamine lake, malachite green lake, Hansa yellow, benzidine yellow, and brilliant carmine 6B.

The pigment can be used in combination with a dye such as an oil soluble azo dye including oil black and oil red, a basic azo dye including bismark brown, an acidic azo dye including blue black HF, and quinone imine dye including nigrosine. Further, it is possible to use a so-called "processed pigment", i.e., a pigment having the surface coated with a resin.

The colorant is added in advance to a thermoplastic resin by means of kneading under heat. Alternatively, the colorant can be added during manufacture of the liquid toner composition of the present invention. Specifically, the colorant can be added before precipitation of the toner particles.

The resin used in the present invention should desirably a thermoplastic resin including, for example, vinyl chloride resin, vinylidene chloride resin, vinyl acetate resin, polyvinyl acetal resin, styrene series resin, methacrylic acid series resin, polyethylene resin, polypropylene resin, fluorine-containing resin, polyamide series resin, polyacetal resin, and saturated polyester resin. It is particularly desirable to use olefin resins having carboxyl groups or ester bonds including, for example, ethylene-vinyl acetate copolymer, partially saponified ethylene-vinyl acetate copolymer, ethylene-acrylic acid copolymer, ethylene-methacrylic acid copolymer, ethylene-acrylic acid ester copolymer, ethylene-methacrylic acid ester copolymer, acrylic acid ester resin, methacrylic acid ester resin, styrene-acrylic acid copolymer, styrene-methacrylic acid copolymer, styrene-acrylic acid ester copolymer, and styrene-methacrylic acid ester copolymer. These resins can be used singly or in the form of a mixture of at least two kinds of resins. Also, these resins can be mixed in an amount of 50 to 99% by weight relative to 50 to 1% by weight of the pigment.

The carrier liquid used in the present invention includes, for example, a linear or branched aliphatic hydrocarbon, alicyclic hydrocarbon and halogenated derivatives thereof. It is also possible to use silicone oils. Specific examples of the carrier liquid used in the present invention include, for example, Isopar G (trade name of a carrier liquid produced by Exxon Inc.), Isopar H (trade name of a carrier liquid produced by Exxon Inc.), Isopar K (trade name of a carrier liquid produced by Exxon Inc.), Isopar L (trade name of a carrier liquid produced by Exxon Inc.), Isopar M (trade name of a carrier liquid produced by Exxon Inc.), Isopar V (trade name of a carrier liquid produced by Exxon Inc.), Shellzole 71 (trade name of a carrier liquid produced by Shell Oil Co., Ltd.), IP1620 (trade name of a carrier liquid produced by Idemitsu Petrochemical Co., Ltd.), IP2028 (trade name of a carrier liquid produced by Idemitsu Petrochemical Co., Ltd.), IP2835 (trade name of a carrier liquid produced by Idemitsu Petrochemical Co., Ltd.), cylooctane, cyclodecane, and TSF451 series (trade name of silicone oils produced by Toshiba Silicone Inc.).

The solvent used in the present invention for dissolving the resin should be capable of dissolving the resin in the heating step and should be substantially incapable of dissolving the resin at room temperature. In the present invention, the solvent is used for controlling the diameter of the precipitated toner particles. Therefore, the SP (Solubility Parameter) value of the solvent is specified in the present invention. It should be noted that a differential SP value (ΔSP) between the SP value of the resin itself and that of the solvent should be as small as possible for diminishing the toner particle diameter. The solvent meeting the particular requirements includes, for example, linear or branched aliphatic hydrocarbons, halogenated aliphatic hydrocarbons, aromatic hydrocarbons, aliphatic alcohols and ethers. These solvents can be used singly or in the form of a mixture.

The inorganic fine particles used in the present invention include titanium oxide particles and titanium hydroxide particles. The particle diameter and the specific surface area of these inorganic fine particles, which can be chosen as desired, should desirably fall within a range of between 2 nm and 500 nm in terms of the primary particle diameter and within a range of between 20 m²/g and 500 m²/g, respectively.

In order to control the dispersion capability or affinity with the resin of the inorganic fine particles, these inorganic fine particles have the surface treated with an organic material or hydroxide.

Specific surface-treated titanium-based inorganic fine particles used in the present invention include, for example, STR series particles produced by Sakai Kagaku Kogyo K.K. such as STR-40, STR-60, STR-65, STR-80, STR-100, and C-11 produced by Ishihara Sangyo Kaisha Ltd.

Further, an antistat and/or a dispersant can be added to the liquid toner composition of the present invention. The antistat used in the conventional developing agent can be used in the present invention. For example, the antistat used in the present invention include nigrosine series dyes; metal soaps such as manganese naphthenate, calcium naphthenate, zirconium naphthenate, cobalt naphthenate, iron naphthenate, lead naphthenate, nickel naphthenate, chromium naphthenate, zinc naphthenate, magnesium naphthenate, manganese octylate, calcium octylate, zirconium octylate, iron octylate, lead octylate, cobalt octylate, chromium octylate, zinc octylate, magnesium octylate, manganese dodecylate, calcium dodecylate, zirconium dodecylate, iron dodecylate, lead dodecylate, cobalt dodecylate, nickel dodecylate, chromium dodecylate, zinc dodecylate and magnesium dodecylate; alkylbenzene sulphonates such as calcium dodecylbenzene sulphonate, sodium dodecylbenzene sulphonate, barium dodecylbenzene sulphonate; phospholipids such as lecithin and cephalin; and organic amines such as n-decyl amine. These antistats can be used singly or in combination.

It suffices to use the antistat in an amount sufficient for obtaining an antistat effect. In general, the amount of the antistat should be 0.5 to 50% by weight, preferably 1 to 30% by weight, based on the amount of the solid components of the liquid toner composition.

The dispersant used in the present invention should desirably be an anionic or nonionic surfactant having ethylene oxide added thereto as a hydrophilic group. When it comes to the anionic surfactant, it is desirable to use a phosphate ester of a higher alcohol ethylene oxide adduct, which is classified as a phosphate ester. On the other hand, the nonionic surfactant used in the present invention includes, for example, a higher alcohol ethylene oxide adduct, alkylphenol fatty acid ester ethylene oxide adduct, fatty acid ethylene oxide adduct, polyhydric alcohol fatty acid ester ethylene oxide adduct, higher alkylamine ethylene oxide adduct, fatty acid amide oxide adduct, ethylene oxide adduct of fat and oil, and polypropyleneglycol ethylene oxide adduct. These surfactants can be used singly or in combination. It is desirable to add the dispersant in an amount of, generally, 0.5 to 80% by weight and, preferably, 1 to 50% by weight, based on the amount of the solid components of the liquid toner composition.

In developing an electrostatic image formed on the surface of a photosensitive body in an electrophotographic system using a liquid toner composition, a good dispersion capability of the toner particles permits a good resolution, leading to a high quality of the picture image developed on the photosensitive surface.

On the other hand, where the picture image (toner layer) on the photosensitive surface is transferred onto a supporting sheet such as a paper sheet, it is desirable for the toner particles to exhibit a high agglomerating force so as to enable the toner layer to have a high viscosity. It should be noted that, where the toner layer has a high viscosity, it is possible to suppress collapse of the picture image and flow of the toner particles in the transferring step, leading to an improved quality of the picture image transferred onto the supporting sheet.

The liquid toner composition of the present invention exhibits an ER property, as already pointed out. It should be noted that, in the developing step, the concentration of the solid components of the composition is low so as to permit the toner particles in the composition to exhibit a high dispersion capability. It follows that a picture image of a high quality can be formed on the photosensitive surface. On the other hand, an electric field is applied for the transferring purpose to the picture image (toner layer) formed on the photosensitive layer after the developing step. What should be noted is that the toner layer noted above has a high concentration of the solid components. When the electric field is applied to the particular toner layer, an agglomerating force is instantly generated among the toner particles by an ER effect so as to increase the viscosity of the toner layer, with the result that it is possible to suppress collapse or deformation of the picture image in the transferring step. Incidentally, the term "ER effect" noted above denotes the effect that the agglomerating force among the toner particles dispersed in a liquid carrier is increased by the electric field application so as to increase the apparent viscosity of the liquid composition.

It has been found that a liquid toner composition having an ER property can be obtained by adding the inorganic fine particles defined in the present invention in the manufacturing process of the composition. Particularly, it has been found desirable to add the inorganic fine particles in an appropriate stage falling within a period between the starting step and the step immediately before precipitation of the toner particles. It is considered reasonable to understand that the inorganic fine particles are attached to or impregnated in at least the surface region of the toner particle so as to produce the ER effect.

As described above in detail, the present invention provides a liquid toner composition containing toner particles which do not exhibit a high agglomerating force and are excellent in dispersion capability during storage and development of the composition, and which exhibit an increased agglomerating force in the transferring step so as to suppress collapsing and flow of the picture image, leading to an improved picture image. The present invention is also intended to provide a method of manufacturing the particular liquid toner composition.

Let us describe some Examples of the present invention. The expressions "parts" and "%" in the following description represent "parts by weight" and "% by weight", respectively.

### Example 1

A dispersion of inorganic fine particles was prepared in the first step. Specifically, 900g of C-11 (trade name of hydrated titanium oxide manufactured by Ishihara Sangyo Kaisha Ltd.) was dispersed in 3,000g of a mixed solvent consisting of 48% of Isopar L (trade name of a carrier liquid produced by Exxon Inc.), 32% of toluene manufactured by Katayama Chemical Co., Ltd. and 20% of ethanol manufactured by Katayama Chemical Co., Ltd. using a dispersing apparatus "Dynomil KDL-Pilot type" having 1.4 liters of a pulverizing chamber, which is sold by Shinmaru Enterprises Inc.

Then, put in a container equipped with a stirrer, a thermometer and a reflux condenser were 43g of the resultant dispersion of the inorganic fine particles, 3750g of the mixed solvent noted above, 50g of "Dumiran C-2280 (trade name of a partially saponified ethylene-vinyl acetate copolymer manufactured by Takeda Yakuhin Inc.), and 10g of "C.I. Pigment Blue" (trade name of phthalocyanine blue manufactured by Dainichi Seika Kogyo K.K.), which was subjected in advance to a dispersion treatment within a mixed solvent using "Dynomil" noted above. The resultant mixture was kept stirred for 30 minutes at 70°C to permit Dumiran C-2280 to be dissolved completely, followed by cooling to room temperature so as to precipitate toner particles. Further, the mixed solvent of the toner particle dispersion was replaced by Isopar L, followed by adding zirconium naphthenate as an antistat so as to charge the toner particles positive.

Table 1 shows the properties of the resultant liquid toner composition and the result of evaluation of the picture image quality. The toner particle diameter given in Table 1 denotes a volume-based median diameter measured by a laser diffraction/scattering type particle size distribution meter LA-700 manufactured by Horiba Seisaku-sho Ltd. The zeta potential in Table 1 was measured by using LEZA-600 (trade name of a laser zeta static charge gauge manufactured by Otsuka Denshi K.K. Further, the ER property was evaluated by a method shown in Figure using an Ostwald viscometer 1. As shown in Figure, an electrode 2 (copper plate) was connected inside the Ostwald viscometer 1. A liquid toner composition 3 having a toner concentration of 10% was housed in the Ostwald viscometer 1. Further, a bare copper wire 4 having a diameter of 0.2 mm was arranged within the Ostwald viscometer 1 and connected to a high voltage power source 5.

For evaluating the picture image quality, the formed image was printed on a coated paper sheet by using "Mitsubishi Printing System", and the resultant printing was visually evaluated. The image density was measured by using a Mackbeth densitometer.

As apparent from Table 1, a good picture image quality was obtained in Example 1.

### Comparative Example 1

A liquid toner composition was prepared as in Example 1, except that a dispersion of the inorganic fine particles was not used for preparing the composition. Table 1 also shows the properties of the resultant liquid toner composition and the result of evaluation of the picture image quality. As apparent from Table 1, the picture image quality for Comparative Example 1 was inferior to that for any of Examples 1 and 2.

### Example 2

Put in a container equipped with a stirrer, a thermometer and a reflux condenser were 3,750g of a mixed solvent, 50g of Dumiran C-2280, i.e., a partially saponified ethylene-vinyl acetate copolymer referred to previously, and 10g of a 57 : 1 mixture of brilliant carmine 6B and C.I. Pigment, said mixture being manufactured by Dai-Nichi Seika Kogyo Inc. and subjected in advance to a dispersion mixing in a solvent by using "Dynomil" referred to previously. The mixed solvent noted above consisted of 48% of Isopar L, 32% of toluene, and 20% of ethanol. The resultant mixture was kept stirred for 30 minutes at 70°C. After Dumiran C-2280 was completely dissolved, 43g of the inorganic fine particle dispersion prepared as in Example 1 was added to the resultant solution, followed by cooling the mixture to room temperature so as to allow the toner particles to be precipitated. The mixed solvent of the toner particle dispersion was replaced by Isopar L, and zirconium octylate was added as a charging agent to the dispersion so as to charge the toner particles positive. Table 1 also shows the properties of the resultant liquid toner composition and the result of evaluation of the picture image quality. As apparent from Table 1, the picture image quality for Example 3 was found to be excellent as in Example 2.

### Comparative Example 2

A liquid toner composition was prepared as in Example 3, except that the mixed solvent of the inorganic fine particle dispersion, which was added before precipitation of the toner particles, was replaced by Isopar L, followed by adding a charging agent. Table 1 also shows the properties of the resultant liquid toner composition and the result of evaluation of the picture image quality. As apparent from Table 1, it was impossible to obtain a satisfactory picture image quality in Comparative Example 2.

As described above, the liquid toner composition of the present invention can be used quite satisfactorily in an picture image output machine of an electrophotographic system. Specifically, the toner particles in the composition are dispersed sufficiently when the composition is used for developing an electrostatic image formed on a photosensitive body surface, leading to an excellent quality of the image developed on the photosensitive body. On the other hand, when the image developed on the photosensitive body is transferred onto a supporting sheet, the viscosity of the toner layer in the picture image portion is rapidly increased by the ER effect. It follows that the collapse of the picture image and flow of the toner particles in the transfer step can be suppressed, leading to output of a high quality picture image.

## Claims

1. A liquid toner composition, characterized in that said toner particles containing a colorant and a resin as main components are dispersed in a carrier liquid, titanium oxide or titanium hydroxide is attached to or contained in a surface region of said toner particles, and the surface of said titanium oxide or titanium hydroxide is treated with an organic substance or a hydroxide.

2. A method of manufacturing a liquid toner composition, characterized by comprising the step of heating, dissolving, mixing and dispersing a thermoplastic resin in a solvent that permits dissolving said thermoplastic resin when heated and is substantially incapable of dissolving the thermoplastic resin at room temperature, said solvent having a solubility parameter (SP) value adjusted for controlling the diameter of the toner particle based on a difference in SP value between the thermoplastic resin itself and the solvent, followed by cooling to permit the toner particles to be precipitated, wherein inorganic fine particles are added by at latest the stage immediately before initiation of the toner particle precipitation.

## Patentansprüche

1. Flüssigtonermischung, **dadurch gekennzeichnet, dass** die Tonerpartikel mit einem Farbstoff und einem Harz als Hauptkomponenten in einer Trägerflüssigkeit gelöst sind, Titanoxid oder Orthotitansäure in einem Oberflächenbereich der Tonerpartikel angeheftet oder enthalten ist, und die Oberfläche des Titanoxids oder der Orthotitansäure mit einer organischen Substanz oder einem Hydroxid behandelt ist.

2. Verfahren zur Herstellung einer Flüssigtonermischung, **gekennzeichnet durch** die Schritte von Heizen, Lösen, Mischen und Dispergieren eines thermoplastischen Harzes in einer Lösung, die das Lösen des thermoplastischen Harzes ermöglicht, wenn es erwärmt und im wesentlichen ungeeignet zur Lösung des thermoplastischen Harzes bei Raumtemperatur ist, wobei die Lösung einen Löslichkeitsparameter (SP) Wert hat, der geeignet zur Steuerung des Durchmessers der Tonerpartikel basierend auf einer Differenz des SP-Wertes zwischen dem thermoplastischen Harz selbst und der Lösung ist, gefolgt durch Abkühlen, um ein Ausfällen der Tonerpartikel zu ermöglichen, wobei anorganische Feinteilchen spätestens in der Stufe direkt vor Einleiten der Tonerpartikelabscheidung hinzugefügt werden.

## Revendications

1. Composition de toner liquide, caractérisée en ce que lesdites particules de toner contenant un colorant et une résine comme composés principaux sont dispersées dans un liquide véhicule, de l'oxyde de titane ou de l'hydroxyde de titane est fixé à ou contenu dans une région de surface desdites particules de toner, et la surface dudit oxyde de titane ou de l'hydroxyde de titane est traitée avec une substance organique ou un hydroxyde.

2. Procédé de fabrication d'une composition de toner liquide, caractérisé en ce qu'il comporte les étapes de chauffage, dissolution, mélange et dispersion d'une résine thermoplastique dans un solvant qui permet de dissoudre ladite résine thermoplastique lorsqu'elle est chauffée et est sensiblement incapable de dissoudre la résine thermoplastique à température ambiante, ledit solvant ayant une valeur de paramètre de solubilité (SP) ajustée pour contrôler le diamètre des particules de toner sur la base de la différence de valeurs SP entre la résine thermoplastique elle-même et le solvant, suivies par le refroidissement pour permettre aux particules de toner de précipiter, dans lequel de fines particules inorganiques sont ajoutées au plus tard à l'étape immédiatement avant l'initiation de la précipitation des particules de toner.
